

June 9, 1936.

A. J. MARINO

2,043,549

METHOD OF COATING FERROUS STRIP MATERIAL

Filed March 17, 1933



Anthony J. Marino  
INVENTOR

Frank P. Newlin  
ATTORNEY

## UNITED STATES PATENT OFFICE

2,043,549

## METHOD OF COATING FERROUS STRIP MATERIAL

Anthony J. Marino, Union City, N. J., assignor to  
 Gilby Wire Company, Newark, N. J., a corpora-  
 tion of New Jersey

Application March 17, 1933, Serial No. 661,303

4 Claims. (Cl. 148—17)

The invention relates to a method of coating ferrous strip material, and more particularly to the application of a thin coating of carbon to the surfaces of a base strip or strand without so 5 hardening it as to impair its properties of malleability or ductility.

In the production of thermionic tubes for use in radio sets, the use of a bright metal anode or plate has been found to result in overheating of 10 the anode or plate, with a consequent interference with the constant capacity of the tube, due to the tendency of the electrons emitted from the cathode to adhere to, or accumulate upon, the surface of the plate. To overcome this difficulty, 15 attempts have been made to apply a coating of carbon to nickel or nickel alloys, but the methods employed are such as to require excessively high temperatures, and the product not only is so expensive as to materially increase the cost of 20 the tubes, but contains other objectionable characteristics so far as reliability in the action of different tubes is concerned.

Attempts to apply a carbon coat to soft iron or steel strip or wire have, prior to my invention, 25 been unsuccessful because, by the methods employed, the application of the carbon to the base material has resulted in the chemical modification of the structure of the ferrous material at its surface resulting in the hardening thereof in a 30 manner to preclude the subsequent forming or drawing operations necessary to give to the material the form required to adapt it for use in an electron tube, or for other purposes.

I have discovered that a permanent, thin coating of carbon may be applied to a base consisting 35 of a strip or wire of soft iron or steel by subjecting it to an elevated temperature in the presence of an oxidizing medium resulting in the oxidation of the surface of the iron or steel, subsequently 40 reducing the temperature of the ferrous material of the strip or wire, and then subjecting the oxidized strip or wire to an elevated temperature in the presence of a gas rich in carbon.

In the practice of the process, I have found it 45 necessary, to avoid the hardening of the surface of the iron or steel, to keep within a narrow temperature range during the oxidizing and the carbonization stages, and to control the temperatures attained by the base strip or wire by the 50 speed at which the same travels while subjected to the elevated temperatures above referred to.

The success of the method or process is dependent largely upon the factors of time and temperature during, and at which the oxidation step 55 and the carbonization step are performed. The

proper temperatures and the proper time intervals ensure a high degree of uniformity and permanency in the carbon coating throughout the entire length of the strip or wire without any appreciable hardening effect upon the material of 5 the base strip or wire.

The invention consists primarily in a method of coating ferrous strip material consisting in subjecting a strip or wire of soft iron or steel to a temperature of substantially 1200° F. in the 10 presence of an oxidizing medium for a time interval of substantially four minutes, air cooling the strip or wire for an interval of substantially four minutes, and then subjecting the oxidized strip or wire to a temperature of substantially 15 1100° F. in the presence of a gas rich in carbon for a time interval in excess of four minutes; and in such other novel steps and practices as are hereinafter set forth and described, and more particularly pointed out in the claims hereto 20 appended.

In the accompanying drawing, I have illustrated diagrammatically the method of the invention.

In the drawing, *a* indicates a coil of strip or wire 25 of iron or steel of soft drawing stock. The wire from the coil *a* passes through a furnace *b* in which atmospheric air is permitted to circulate freely. After leaving the furnace *b*, the strip or wire from the coil *a* passes in the presence of an 30 oxidizing medium through a low temperature zone *c*, until it enters a carbonizing furnace *d* charged through a pipe *e* with a gas rich in carbon. The furnace *d* is completely closed, except for substantially gas tight roller gates *f* and *g* 35 at the points where the strip or wire *a* enters and leaves the furnace. Beyond the furnace *b* is a quenching tank *h* for cooling the completed product before collecting it upon the rewind reel *i*, which may be continuously rotated in any 40 desired manner, as by the speed reducing mechanism *j*, to ensure a continuous rate of travel of the strip or wire *a*. Guide rollers *k*, *k*<sup>1</sup>, *k*<sup>2</sup>, *k*<sup>3</sup>, *k*<sup>4</sup>, and *k*<sup>5</sup> are provided to ensure a proper run of 45 the strip or wire.

By reference to the foregoing description, it will be noted that the method is a continuous one, and may be carried on in a manner to ensure substantially uniform time intervals during each step of the method as to every portion of the 50 length of strip or wire. This results in uniformity throughout the product, which is highly desirable from the standpoint of manufacturers employing the product.

Referring more particularly to the procedure 55

followed in the practice of the method of the invention, a temperature of approximately 1200° F. is maintained in the oxidizing furnace *b*, and a relatively lower temperature, substantially 1100° F. is maintained in the carbonizing furnace *d*. The length of the oxidizing furnace *b* is approximately 4 feet; the length of the low temperature zone intermediate the furnaces *b* and *d* is approximately 4 feet, and the length of the carbonizing furnace *d* is approximately twice that of the oxidizing furnace.

The means actuating the rewind reel is so geared as to impart a substantially uniform speed to the strip or wire of one foot per minute. Any desired mechanical expedients for ensuring a uniform speed of the strip or wire may be employed.

The length of the furnaces and the speed of the strip or wire are time factors with which, at the temperatures stated, a thin strip, approximately .005 of an inch in thickness, is oxidized and coated with carbon to the desired extent.

Oxidizing apparently occurs while the strip or wire is passing through both the furnace *b* and the low temperature, air cooling zone *c*.

The desired reactions result from the temperatures to which the material is subjected and the time during which they are subjected to such temperatures. These factors are not constant, to the extent that they must be varied in proportion to the cross sectional area of the material. This variation may be secured with materials of greater cross sectional area than stated by using furnaces of greater length, by reducing the speed of the material or by increasing the temperature in the furnaces within a small range. I have herein given an example of time and temperatures which I have found give excellent results when the material being coated is substantially pure commercial, or Swedish iron.

The oxidizing medium used is ordinary atmospheric air. In the furnace *d*, I may use natural gas, producer gas or other gases rich in hydrocarbons, which, if desired, may be enriched as compared with the normal product in the manner usually employed for producing enriched gas, to wit: the introduction of hydrocarbons during the production or consumption of the gases.

Water may be used in the quenching bath *h*, the purpose of this bath being merely to reduce the temperature of the material before re-coiling same.

The time and temperature factors are such as to ensure the deposit of a permanent carbon coating on the surface of the base strip or wire *a*, which apparently is of uniform thickness and actually incorporated in the structure of the base at the surface thereof. There is no reduction having any appreciable hardening effect upon the iron of the base, and the completed product has substantially the same inherent properties of malleability or ductility as the untreated strip or wire. It may be formed or drawn into any desired shape without the development of surface cracks or checks.

The temperature employed during the carbonization step is vital to the successful practice of the method of the invention, although this temperature is subject to slight variation, as herein referred to, so long as the conditions are such as to ensure a temperature of the ferrous base which is substantially that resulting from the example herein stated. During oxidation alone there can be no material hardening of the base. During carbonization there would be such a hard-

ening, if excessively high temperatures were employed.

The word "permanent" is used herein to mean that the major portion of the coating is so incorporated in the structure of the base at the surface thereof as to resist separation therefrom except by abrasion. Light buffing will have no effect upon the coating, except the removal of a small percentage of the surface carbon.

While I have described the use of the material produced by the method of the invention in the production of thermionic tubes, it is obvious that the uses to which the product is put are immaterial to the invention.

The temperatures attained by the ferrous base are controlling in the practice of the method, and since they are the resultant of the time and temperature factors herein referred to, variation of these temperatures as herein referred to are permissible so long as the resultant temperatures are substantially constant.

Because of the low temperature developed in the carbonizing furnace or chamber, the quenching bath will have no effect in hardening the surface of the product.

Having described the invention, what I claim as new and desire to have protected by Letters Patent, is:—

1. The herein described method of coating ferrous strip material consisting in subjecting a strip or wire of soft iron or steel to a temperature of substantially 1200° F. in the presence of an oxidizing medium for a time interval of substantially four minutes, air cooling the strip or wire for an interval of substantially four minutes, and then subjecting the oxidized strip or wire to a temperature of substantially 1100° F. in the presence of a gas rich in carbon for a time interval in excess of four minutes.

2. The herein described method of coating ferrous strip material consisting in subjecting a strip or wire of soft iron or steel to a temperature of substantially 1200° F. in the presence of an oxidizing medium for a time interval of substantially four minutes, air cooling the strip or wire for an interval of substantially four minutes, then subjecting the oxidized strip or wire to a temperature of substantially 1100° F. in the presence of a gas rich in carbon for a time interval in excess of four minutes, and thereafter passing the strip or wire through a quenching bath.

3. The herein described method of coating ferrous strip material consisting in continuously roving a strip or wire of soft iron or steel successively through an oxidizing medium maintained at substantially a temperature of 1200° F. for a time interval of substantially four minutes, through an air cooling zone for a time interval of substantially four minutes and through a gas rich in hydro-carbon maintained at a temperature of 1100° F. for an interval of substantially eight minutes.

4. The herein described method of coating ferrous strip material consisting in continuously moving a strip or wire of soft iron or steel successively through an oxidizing medium maintained at substantially a temperature of 1200° F. for a time interval of substantially four minutes, through an air cooling zone for a time interval of substantially four minutes and through a gas rich in hydro-carbon maintained at a temperature of 1100° F. for an interval of substantially eight minutes, and passing the strip or wire through a quenching bath.